

March 8, 1960

D. LEWIS, JR., ET AL

2,927,865

COATED HEAT-SEALABLE WRAPPER AND PROCESS OF MAKING SAME

Filed Feb. 24, 1956



Fig 1



Fig 2

INVENTORS  
JOHN S. BARTON  
DAN LEWIS JR.  
BY

*F. Feisler*

ATTORNEY

1

2,927,865

## COATED HEAT-SEALABLE WRAPPER AND PROCESS OF MAKING SAME

Dan Lewis, Jr., and John S. Barton, Camas, Wash., assignors to Crown Zellerbach Corporation, San Francisco, Calif., a corporation of Nevada

Application February 24, 1956, Serial No. 567,588

12 Claims. (Cl. 117—14)

This invention relates to a wrapping material especially adapted for frozen foodstuffs and other products which, while wrapped, are to be kept in below freezing temperatures.

More specifically, this invention relates to the production of a paper wrapper which has been rendered substantially moistureproof by waxing, which is capable of being heat-sealed, but which, when heat-sealed, will maintain a strong bond where such heat-sealing has taken place regardless of subsequent prolonged exposure to sub-freezing temperatures.

While various types of waxed paper have long been employed as food wrappers, and, under certain conditions, have proved thoroughly satisfactory for such use due to the fact that they are capable of being heat-sealed and provide a protective and moistureproof covering as long as the seal is maintained, such wrappers have been found to be very unsatisfactory in the case of foods which must be kept in freezers, or in other refrigerating means, under below freezing temperatures, due to the fact that the wax seal then in all likelihood will fail or delaminate during the handling of the packaged foodstuff. Various waxes and mixes of waxes have been tried out in an attempt to produce a heat-sealable wax paper wrapper in which the seal will resist delamination under exposure to low temperatures, but, to the best of our knowledge, thus far without success.

An object of the present invention is to provide an improved wrapper for foods and the like which will be capable of being heat-sealed and which will maintain such seals under temperatures as low as 10° F.

Another object of the invention is to provide an improved frozen food wrapper which will be substantially moistureproof and thus, when sealed, will enable the food incased therein to maintain its original moisture content while being protected from outside moisture, vapor, or dust as long as the wrapper remains sealed.

An additional object of the invention is to provide an improved wrapper which will have a surface especially adapted for receiving printing ink and thus suitable for printing.

A further object of the invention is to provide an improved wrapper, particularly adapted for frozen foods, which can be produced easily and economically and which will require only conventional equipment in its manufacture.

Briefly, we attain these objects and other advantages by first coating at least one face of a sheet of paper, of suitable weight for use as a wrapper, with a fluid, pigmented coating composition comprising, as its essential ingredients, a finely divided coating pigment and a polyvinyl acetate resin. The coated paper then, after being substantially dried, is supercalendered, with the result that the treated surface is rendered smooth and is particularly receptive to printing ink. Consequently the wrapper at this stage presents a surface which is very suitable for printing. As a final step in the production of the wrapper, the coated paper (after being printed,

2

if a printed wrapper is desired), is given a treatment of wax, either on the coated face alone or on both faces. The resultant coated and waxed sheet presents a finished, glossy surface which is heat-sealable, and, when heat-sealed, will maintain its seal even though exposed over a prolonged period to temperatures as low as 10° F. The important and novel feature of the invention is the fact that, due to some physical interaction between the particular pigmented polyvinyl acetate resin and the film of wax on the bonded surfaces of the base paper sheet, which occurs under the heat-sealing, a tenacious bond is set up between the heat-sealed surfaces and this bond will not delaminate, even under low temperatures, and can be broken only by rupture of the paper sheet.

15 Preferably, in the carrying out of the invention, the paper sheet for the wrapper should have a basis weight of from about 15 pounds to 150 pounds per ream of 3,000 square feet, and a basis weight of from 20 pounds to 35 pounds per ream is considered most satisfactory 20 since the paper then will be heavy enough for customary wrapper use without being unnecessarily heavy. Any of the conventional "beater additives," such as sizing agents, wet-strength resins, fillers, opacifying pigments, etc., may, if desired, be incorporated in the pulp furnish 25 from which the paper sheet is made. It is desirable that the sheet be fairly well sized in order to prevent excessive penetration by the pigmented polyvinyl acetate resin. A pulp furnish consisting of about 80 percent bleached softwood sulfite and about 20 percent hardwood soda 30 pulp has been found to be very suitable for the manufacture of the paper sheet to be employed in the carrying out of this invention.

In the accompanying drawings, which are more or less diagrammatic, Figure 1 is a sectional elevation, 35 drawn to a considerably enlarged scale, of a portion of a frozen food wrapper embodying the present invention; and

Figure 2 is a similar sectional elevation of a food wrapper also made in accordance with the invention, 40 but with both faces of the wrapper waxed.

In the drawings the reference character 10 indicates the paper sheet from which the wrapper is made. The pigmented polyvinyl acetate resin coating applied to the paper sheet is indicated by the reference character 11. 45 After the coating has dried, and the coated surface preferably has been supercalendered and printed (assuming that a printed wrapper is desired), the coated sheet is given a wax treatment. In Figure 1 the film of wax which is applied to the coated face of the paper is indicated by the reference character 12. In Figure 2 both the coated and uncoated faces of the paper have received a thin film of wax, as indicated by the reference characters 13 and 14, respectively. In some instances the waxing of both sides of the sheet may be preferred and 50 this will be a convenience, for example, when the waxing can be accomplished most conveniently by dipping the coated paper in the melted wax. In such case, since both faces of the paper are waxed, the film of wax on each face is preferably slightly thinner than when the 55 wax is confined only to the coated face.

It would, of course, also be possible to carry out the invention by coating both faces of the paper sheet with the pigmented polyvinyl acetate resin and then waxing both coated faces. However, since this is not necessary, 60 this consequently is not the preferred manner of performing the invention.

The essential constituents of the pigmented coating composition are a pigment and a polyvinyl acetate resin adhesive. The materials which comprise these particular constituents for the carrying out of the invention will now 65 be described more fully.

For the pigment constituent several kinds of white

or colored pigments of fine particle size, and various combinations thereof may be used. Examples of these are barium sulfate, calcium carbonate, calcium sulfite, clays, titanium dioxide, etc. If desired, colors or dyes customarily used in color mixes may be admixed therewith to impart to the pigmented composition a particular desired shade. In selecting a particular pigment or pigments, such factors as brightness, opacity, printing qualities of the coated sheet, as well as the compatibility with the polyvinyl acetate resin adhesive must be considered. A combination of 60 to 85 parts by weight of titanium dioxide with 15 to 40 parts by weight of coating clay has been found to be highly satisfactory for employment in this invention. A small amount of dispersing agent should be added for the pigment. Some of the satisfactory dispersants are tetrasodium pyrophosphate, sodium hexametaphosphate, sodium silicate, etc. The proportion of the dispersant should not be too high to prevent flocculation of the pigment in the liquid medium.

The other and essential constituent of the coating composition, namely the polyvinyl acetate resin, is available on the market in form of liquid emulsions of dispersions. We have found that particularly suitable resins for use in combination with the above mentioned pigments are the aqueous polyvinyl acetate emulsions having an average particle size in the range of 0.5-5.0 microns, and preferably 1 to 3 microns, viscosity in the broad range of 5 to 2000 centipoises, and preferably 500-1200 centipoises at 25° C. Such resins provide a strong bond between the heat-sealed areas of the final wrapper upon its exposure to a temperature range of from about 10° F. to about 90° F., the heat sealing operation being carried out at a temperature above the softening point of the polyvinyl acetate resin. Examples of highly satisfactory polyvinyl acetate aqueous emulsions are: "Elvacet 81-900," produced by E. I. du Pont de Nemours and Co., Inc., "Vinac XX," produced by Colton Chemical Co., Cleveland, Ohio, and "Resyn 10 K 04," produced by National Starch Products Co., San Francisco, California.

If desired, a secondary adhesive, a plasticizer for polyvinyl acetate, and a liquid medium may also be used as auxiliary constituents in the coating composition. Any starch or a proteinaceous adhesive customarily used in the coating of papers may be used as a secondary adhesive. Thus unmodified starches, as well as enzyme-converted, oxidized, or otherwise modified starches are satisfactory. A starch particularly suitable for use in admixture with polyvinyl acetate emulsion is a hydroxyethyl ether derivative of corn starch supplied by the Penick & Ford Company, Cedar Rapids, Iowa, under the trademark "Penford Gum 280." The protein adhesives usually employed in paper coating formulations include casein, animal glue, soya, etc. Alpha-protein (isolated soya protein), which is available on the market from many sources, has been found to be a highly satisfactory proteinaceous adhesive for use in the coating composition of this invention.

It will be understood by those skilled in the art that in choosing a secondary adhesive, its compatibility with the polyvinyl acetate resin and with the pigment, its ease of dissolving or forming homogeneous pastes, its film-forming qualities, and other factors must be taken into consideration. We have found that the polyvinyl acetate resin solids in the adhesive composition may be reduced up to about 30% and the secondary adhesive (solids basis) substituted in place thereof without affecting adversely the seal strength of the finished wrapper. At the same time, the secondary adhesive improves to a certain degree, the rub resistance of the pigmented composition coating on the sheet in addition to reducing its cost.

The addition of a certain amount of a plasticizer to the polyvinyl acetate emulsion has been found to improve its effectiveness, mainly in enhancing the smoothness of

the coated face of the paper after supercalendering, and hence its printing qualities. Among the many plasticizers suitable for admixture with the polyvinyl acetate are: 2-ethyl hexyl diphenyl phosphate and ethyl phthalyl ethyl glycolate, both supplied by Monsanto Chemical Co. under the trademarks "Santicizer 141" and "Santicizer E-15," respectively, butylstearate, acetyl tributyl citrate, glycerol monostearate, and others.

A liquid medium, preferably water, may be added to the coating composition for adjustment of its viscosity to a desired level suitable for the coating operation.

The relative amounts of the various ingredients which have been mentioned may be varied within certain limits, as indicated in the following Table I, which shows their broad and preferred range, the proportions being given as parts by weight, solids basis:

TABLE I

|                         | Broad Range | Preferred Range                        |
|-------------------------|-------------|----------------------------------------|
| Pigment                 | 40-90       | 75-87                                  |
| Polyvinyl acetate resin | 10-60       | 13-25                                  |
| Secondary adhesive      | 0-20        | 0-5                                    |
| Plasticizer             | 0-10        | 1.2-2.0                                |
| Dispersant for pigment  | 0.01-1      | 0.1-0.3                                |
| Liquid medium           |             | Sufficient to attain desired viscosity |

As previously mentioned, the inclusion of a secondary adhesive or of a plasticizer is optional. It should be noted, however, that when a secondary adhesive is used to replace a portion of the polyvinyl acetate, the amount of such adhesive in the broad range of Table I should not exceed 20 parts by weight (solids basis) of the total composition solids, in which case the total proportion of the polyvinyl acetate resin and of the secondary adhesive would not be higher than 60 parts by weight (solids basis); in the preferred range of Table I, the amount of the secondary adhesive would not be higher than 5 parts by weight (solids basis), the total proportion of the polyvinyl acetate resin and of the secondary adhesive then being not higher than 25 parts by weight (solids basis).

In preparing the pigmented coating composition, it has been found preferable to dissolve the dispersant in water first, and then to add the pigment so as to produce an aqueous pigment dispersion having a solids content from about 40% to 70%. The mixing should be carried out with vigorous agitation until a homogeneous mixture is obtained. A predetermined quantity of polyvinyl acetate emulsion is then added slowly to the aqueous pigment slurry and mildly stirred until a uniform mixture is produced. When a plasticizer is used, it is admixed first with the polyvinyl acetate. Water or other suitable liquid media may be added to the fluid pigmented coating mixture so that its final viscosity will be adjusted within a broad range of 50-5000 centipoises, and preferably between 250 and 1500 centipoises at 25° C.

The secondary adhesive, if used, is either dissolved or dispersed in a liquid medium, e.g. water, with heating and/or addition of alkali, in accordance with conventional procedures employed in the preparation of starch or protein adhesives used in paper coating operation. It is preferred that the quantity of water used be such as to produce a concentration of solids in the range of 10% to 25%. The secondary adhesive may be either mixed with the polyvinyl acetate resin or added directly to the pigment slurry.

The pigmented coating composition may be applied to the paper by any conventional paper coating procedure, such as kiss-roll, air-knife, brush, size-press, doctor-blade, etc. Care should be taken, however, that the coating be applied over the entire surface of the paper in such a manner as to produce a continuous film of uniform weight ranging broadly from 0.5 to 6 lbs./ream, and preferably 1.5 to 3.0 lbs. (solids basis) per ream of 3000 square feet.

During the coating operation it may be desirable to reduce the foaming of the coating composition. Accordingly, a small amount of a suitable defoamer, usually about 0.05% based on the solids of the composition may be incorporated thereto. Satisfactory defoamers are: octyl alcohol, silicones, esters of fatty acids, etc.

The coated paper is then substantially dried at a temperature between 212° F. and 300° F., preferably between 250° F. and 275° F. by hot air or by passing it over one or more drum driers, or in any other suitable manner. Care should be exercised, however, that the period of time necessary for drying and the drying temperature be so adjusted as to produce a coated paper having from about 4% to 6% moisture content.

After the coated paper is dried, it is subjected to a calendering operation to impart thereto a smooth surface desirable for printing. This operation is carried out by first dampening the paper uniformly by any suitable means, such as a spray of water, to increase its moisture content to about 7%-12%, and preferably 8%-10%, and then passing it through either the entire conventional calender stack or a part thereof if a finish requiring a lesser calendering action is desired. The calender rolls may be either cold or internally heated to a surface temperature up to about 300° F., but preferably not exceeding about 200° F. During its passage through the calender stack, the paper is subjected to a controlled pressure which may vary from about 500 to 2000 pounds per linear inch, depending on the desired ultimate characteristics of the sheet. Satisfactory results were obtained by supercalendering a 30 lb./ream coated sheet of paper with a pressure between 1200 and 1300 pounds per linear inch.

The coated and supercalendered paper may be next printed, if desired, by any of the conventional printing processes, such as rotogravure, letter-press, multicolor offset, etc. The coated surface of the paper is highly satisfactory for printing operation, as it is smooth and has a good affinity for printing inks.

The coated paper, either printed or unprinted, is then waxed by any of the well-known procedures of making papers waxed on either one side or both sides thereof. As indicated above, the wax may be applied only to the coated surface of the paper. This may be accomplished by depositing a film of wax from aqueous emulsion, solvent solution, or from molten bath. Preferably, and generally more conveniently, however, the coated paper is made to pass through a bath of molten wax, then between a pair of squeeze rolls to remove excess of wax, and finally through a chilling bath, and as a result both sides of the paper will be covered with a thin film of wax. The amount of wax necessary to obtain a film of adequate thickness for satisfactorily carrying out the invention may vary from about 8 pounds to 25 pounds per ream (3000 square feet) for both sides of paper, depending on the type of paper used and its basis weight. For a paper having a basis weight of 20 to 35 pounds/ream, the amount of wax ranging from 10 to 15 pounds/ream for both sides of the paper, is generally sufficient.

The term "wax," as used herein, includes such waxes or wax-like materials which give a flexible, non-blocking, heat-sealable film characterized by a good moisture-vapor transmission resistance, and which are capable of producing in conjunction with the hereinabove described pigmented coating a strong heat-seal bond, resistant at sub-freezing temperatures, as low as 10° F.

Particularly suitable in achieving a bond of such strength are wax compositions containing a relatively small amount of polyethylene. As is well known, polyethylene is produced commercially by polymerization of ethylene at high or low pressure. Polyethylene is also available as an irradiated or chlorosulfonated material. Although the molecular weight of the polyethylene may vary to a large extent, a material satisfactory for incorporation into the wax compositions of this invention may

have a molecular weight in the range of 1,500-35,000, and preferably between 3,000 and 20,000.

The two types of waxes which are customarily used in the manufacture of waxed papers are the paraffin wax having a melting point range in the broad range of about 120° F.-200° F., and the preferred range 130° F.-160° F., and the microcrystalline wax having a broad melting point range of about 120° F.-170° F., and preferred range 140° F.-160° F. The combinations thereof in various proportions are also widely employed.

Although other wax materials possessing the hereinabove specified characteristics are equally satisfactory for application over the surface of the paper in the carrying out of this invention, the following Table II shows the most satisfactory wax compositions and proportions of their constituents expressed in percentages by weight.

TABLE II

| 20                        |      | Broad Range | Preferred Range |
|---------------------------|------|-------------|-----------------|
| Paraffin wax.....         | 0-99 | 50-80       |                 |
| Microcrystalline wax..... | 0-99 | 15-45       |                 |
| Polyethylene.....         | 1-40 | 5-15        |                 |

In preparing the wax compositions containing the polyethylene, the wax is usually melted and the predetermined quantity of polyethylene, preferably in finely divided form is added thereto and stirred until dissolved. The resultant wax composition is then ready for use in the waxing operation. The coated and waxed paper may be wound in roll form for ease in handling, shipping, and application.

When a frozen food article is to be wrapped and sealed, a sheet of the coated and waxed paper of adequate size for the package is used and placed so that the coated and waxed side of the sheet will form the outside of the package. The overlapping marginal portions of the wrapping sheet and the closing folds in the same are so arranged that the coating and the wax will be in between the plies to be sealed. The sealing is then accomplished by the application of light pressure and heat for a short period of time sufficient to produce a strong bond. Although what actually transpires to produce the resulting strong bond with the heat-sealing is not entirely understood, it is evident that some physical interaction of the pigmented coating composition with the wax composition and with the two opposed paper surfaces takes place under the influence of the sealing heat and pressure. It has been found that the heat-sealing operation should be carried out at a temperature above the cloud point (ASTM designation D97-47) of the wax composition, preferably at least 10° F. above such cloud point of the wax composition, under which conditions the polyethylene, if present in the wax composition, will be substantially dissolved therein. Furthermore, it has been found to be important that the temperature at which the heat-sealing takes place should be above the softening point of the polyvinyl acetate resin. This is further evidence that some physical interaction between the constituents does occur and is an important factor. Extensive tests have shown that the strength of the bond produced by such heat-sealing is such that it is impossible to pull the bonded areas apart except by rupturing the paper. In other words, whatever the exact nature of the interaction between the constituents may be, no delamination occurs after such interaction is produced by the heat-sealing. Such sealed packages have been tested by being stored for prolonged periods in temperatures around 10° F. without any delaminating or failure of the seals taking place as a result of pulling the bonded areas apart.

The following are some specific examples of the carrying out of the invention. In these examples the proportions are given as parts by weight, solids basis. It is

7  
to be understood, of course, that the invention is not limited entirely to these specific examples.

*Example 1*

|                                                |       |
|------------------------------------------------|-------|
| The pigmented coating was composed as follows: | 5     |
| Pigment                                        | 50    |
| Polyvinyl acetate resin                        | 50    |
| Dispersant                                     | 0.15  |
| Water                                          | 41 10 |

The pigment was composed of 33.5 parts by weight of titanium dioxide "Titanox RA-50," supplied by Titanium Pigment Corp., New York, New York, and 16.5 parts by weight of coating clay "X-43," supplied by J. M. Huber Corp., New York, New York. The polyvinyl acetate resin was Vinac XX, supplied by Colton Chemical Co., Cleveland, Ohio, in form of an aqueous emulsion containing 55-57% solids, having a mean particle size of 1 micron, viscosity at 25° C. in the range of 900-1200 centipoises, and specific gravity at 25° C. of 1.11. (The temperature at which a dry film of this polyvinyl acetate resin begins to soften is 185° F. to 195° F.) The dispersant was tetrasodium pyrophosphate, readily available on the market from many sources.

The dispersant was first dissolved in the 41 parts of water and the two pigments were added thereto gradually and stirred vigorously until a homogeneous dispersion was obtained. The polyvinyl resin was then added slowly to the slurry and stirred mildly until a uniform mixture was produced. The final viscosity of the adhesive was 1200 centipoises at 25° C.

The paper used had a basis weight of 30 pounds per ream (3000 square feet) and was made of a pulp furnish composed of 80% coniferous bleached sulfite and 20% deciduous soda pulp, to which pulp furnish were added about 10% of titanium dioxide filler and 1.1% rosin size precipitated onto the fibers with papermaker's alum, both based on the dry weight of pulp. This paper was uniformly coated on one side thereof with the above coating composition. The coated paper was then passed through a hot-air oven at about 260° F. in such a manner as to leave therein about 5% moisture content. The weight of the dry coating film was 2.5 pounds per ream of paper.

The paper was next supercalendared, by first dampening it with a water mist to increase its moisture content to about 9%, and then passing it between the calender rolls heated to about 190° F., the pressure in each nip being about 1250 pounds per linear inch. The supercalendared paper was then printed on the coated side by 50 the conventional rotogravure process.

Finally the paper was waxed on both sides in a conventional wax coating equipment using a wax composition consisting of 60% of a paraffin wax having a melting point in the range of about 140° F.-145° F., 35% of a micro-crystalline wax having a melting point in the range of about 145° F.-150° F., and 5% of a polyethylene polymer having a molecular weight of about 19,000. After the two waxes had been melted, the polyethylene, in finely divided form, was added thereto and the mixture was stirred until the polyethylene was dissolved. The cloud point of this wax composition was 188° F.-190° F. The paper having a film of molten wax on each side thereof, was then passed through a chilling bath to solidify the wax. The total amount of wax applied on both sides of the paper was about 12 pounds per ream.

A sheet of this finished wrapper was employed for wrapping a package of frozen foodstuff, the coated and printed side of the wrapper constituting the outside surface of the wrapped package. The marginal portions and the end-folds of the wrapper were arranged in such a manner that the surface coated with the pigmented coating and wax was in opposed relationship with the surface having only the wax thereon. The heat-sealing operation was carried out using a conventional sealer, the platens of which

were heated to 225° F. Slight pressure was applied between the hot platens for a very brief period of time (actually about 2 seconds) sufficient to produce a strong bond between the heat-sealed areas of the wrapper.

The heat-sealed package produced in this way was stored in a freezer at a temperature of 10° F. for a period of five weeks. At the end of this period, the bond between the heat-sealed areas was still very strong, and no delamination of these areas occurred.

8  
*Example 2*

The pigmented coating had the following composition:

|                         |       |
|-------------------------|-------|
|                         | Parts |
| Pigment                 | 81    |
| Polyvinyl acetate resin | 17    |
| Plasticizer             | 1.7   |
| Dispersant              | 0.24  |

Water to adjust final viscosity to 200 centipoises at 25° C.

The pigment was composed of the same titanium dioxide and coating clay, as in Example 1, but used in the ratio of 2 to 1, respectively. The polyvinyl acetate resin and the dispersant were also the same as in Example 1. The plasticizer for the polyvinyl acetate resin was 2-ethyl hexyl diphenyl phosphate, sold by the Monsanto Chemical Co. under the trademark "Santicizer 141."

The above ingredients were intermixed in the same manner as in Example 1, however, the plasticizer was added to the resin first, and the plasticized resin was then mixed with the pigment slurry.

The same paper as described in Example 1 was coated with the above composition, then dried, supercalendared, 35 printed, and waxed in the manner set forth in Example 1. The proportions of the ingredients in the wax composition were: 40% paraffin wax, 50% microcrystalline wax, and 10% polyethylene.

The wrapper formed in accordance with this example 40 proved highly satisfactory for packaging frozen foodstuffs, as the strength of its heat-sealed bond had essentially the same characteristics as that of the wrapper of Example 1.

9  
*Example 3*

The pigmented coating had the following composition:

|                         |       |
|-------------------------|-------|
|                         | Parts |
| Pigment                 | 81    |
| Polyvinyl acetate resin | 10.2  |
| Secondary adhesive      | 6.8   |
| Plasticizer             | 1.7   |
| Dispersant              | 0.24  |

Water to adjust final viscosity to 750 centipoises at 25° C.

55 The pigment and the dispersant were the same as in Example 2. The polyvinyl acetate resin was "Elvacet 81-900," supplied by the E. I. du Pont de Nemours Co., in form of an aqueous emulsion containing 55-57% solids, having a mean particle size of 3 microns, viscosity at 25° C. in the range of 800-1000 centipoises, and specific gravity at 25° C. of 1.19. The secondary adhesive was alpha-protein (isolated soya protein) solution, prepared by adding 4 parts of the protein to sufficient water to form a 15% aqueous slurry, heating the slurry to 38° C., adding 0.5 parts of 28% ammonium hydroxide solution to solubilize the protein, and mixing until the protein was dissolved. The plasticizer was butyl stearate.

In preparing the coating composition, the protein solution was added to the aqueous pigment dispersion, then the polyvinyl acetate emulsion containing the plasticizer was added thereto and mixed until a uniform mixture was obtained.

The same paper as described in Example 1 was coated with the above composition, then dried, supercalendared, 70 printed, and waxed in the same manner as set forth in

Example 1. The proportions of the ingredients of the wax composition were slightly modified, however, as follows: 60% paraffin wax, 32.5% microcrystalline wax and 7.5% polyethylene.

The wrapper produced according to this example had the same excellent properties as that of Example 1.

*Example 4*

The pigmented coating had the following composition:

|                         | Parts |
|-------------------------|-------|
| Pigment                 | 81    |
| Polyvinyl acetate resin | 13.6  |
| Secondary adhesive      | 3.4   |
| Plasticizer             | 1.7   |
| Dispersant              | 0.24  |

Water to adjust final viscosity to 2500 centipoises at 25° C.

The pigment consisted of titanium dioxide and coating clay as described in Example 1, but employed in the ratio of 4:1 respectively. The polyvinyl acetate resin was "Vinac XX," the plasticizer was "Santicizer 141," and the dispersant was the tetrasodium pyrophosphate, all previously mentioned. The secondary adhesive was a hydroxyethyl ether derivative of corn starch, produced by the Penick & Ford Co., under the trademark "Penford Gum 280." It was used in form of a solution prepared by admixing the 3.4 parts of the starch in sufficient water to produce about 25% solids content, and heating at 180° F. with agitation until dissolved.

The above ingredients were intermixed in the manner described in Example 3. The same paper as described in Example 1 was coated with the above coating composition, then dried, supercalendered and waxed in the same manner as set forth in Example 1. The wax composition used in this example consisted of 85% paraffin wax, 13.5% microcrystalline wax, and 1.5% polyethylene, the characteristics of the three ingredients having been previously mentioned.

The coated and waxed wrapper had the same properties as that of Example 1.

In Example 1 the platens with which the heat-sealing of the wrapper was accomplished were heated to 225° F. and the time during which the wrapper was in contact with the heated platens was about 2 seconds. The platens could be heated to a higher temperature and the contact time correspondingly reduced. It will be understood, of course, that the temperature of the platens does not mean the temperature to which the pigmented coating and wax are raised during the heat-sealing since the contact period must be of sufficiently short duration to prevent excessive heating of the coating on the wrapper. Thus in commercial operation it has been found to be practical to have the temperature of the platens as high as from 360° F. to 440° F., but the contact time is then carefully restricted to about one-half of a second.

The glossy, heat-sealable, waxed surface of the wrapper of this invention is non-cohesive and non-tacky at normal room temperature, so that the wrapper may be handled or shipped in roll form without any special precautions. The superior printing qualities of the coated surface combined with the advantageous heat-sealing characteristics, imparted by both the coating and the wax film, give as a result a highly satisfactory frozen food paper wrapper possessing the desired feature of being capable of forming a bond at the heat-sealed areas of such a strength that it will not break or delaminate when exposed to sub-freezing temperatures as low as about 10° F. Furthermore, the wrapper is pliable, has a very low moisture-vapor transmission rate, and good physical strength properties.

We claim:

1. The process of making a heat-sealable paper wrapper for use in wrapping frozen foodstuffs, which comprises coating an entire surface of a paper suitable for use as a

wrapper with a quantity of a liquid, pigmented coating composition consisting essentially of a homogeneous mixture of from 40 to 90 parts by weight of a finely divided coating pigment and from 10 to 60 parts by weight, solids basis, of polyvinyl acetate resin, substantially drying the coating so as to produce a continuous film ranging from 0.5 to 6 pounds per ream of 3,000 sq. ft. of the paper, supercalendering the coated paper, and covering the entire coated surface of the paper with a flexible, non-blocking

5 film of wax, the amount of applied wax being sufficient to form with the pigmented polyvinyl acetate coating, upon heat-sealing, a strong bond which will resist delamination at temperatures as low as about 10° F., when the wrapper is heat-sealed at a temperature high enough to melt said wax and soften the polyvinyl acetate resin.

2. The process of claim 1 wherein the wax is selected from the group consisting of paraffin wax, microcrystalline wax, and combinations thereof, and contains up to 40% by weight of polyethylene.

3. The process of making a heat-sealable paper wrapper for use in wrapping frozen foodstuffs, which comprises coating an entire surface of a paper suitable for use as a wrapper with a quantity of a liquid, pigmented coating

25 composition consisting essentially of a homogeneous mixture of from 75 to 87 parts by weight of a finely divided coating pigment and from 13 to 25 parts by weight, solids basis, of polyvinyl acetate resin, substantially drying the coating so as to produce a continuous film ranging

30 from 0.5 to 6 pounds per ream of 3,000 sq. ft. of the paper, supercalendering the coated paper, and covering the entire coated surface of the paper with a flexible, non-blocking film of wax, the amount of applied wax being sufficient to form with the pigmented polyvinyl acetate

35 coating, upon heat-sealing, a strong bond which will resist delamination at temperatures as low as about 10° F. when the wrapper is heat-sealed at a temperature high enough to melt said wax and soften the polyvinyl acetate resin.

4. The process of claim 3 wherein the pigmented coating composition also includes a plasticizer for the polyvinyl acetate in the amount of from 1.2 to 2.0 parts based on the dry weight of said composition and the wax contains up to 15% by weight of polyethylene.

5. The process of making a heat-sealable paper wrapper for use in wrapping frozen foodstuffs, which comprises coating one entire surface of a paper suitable for use as a wrapper with an aqueous, pigmented coating composition, having a viscosity of 50-5000 centipoises and consisting essentially of a homogeneous mixture of from 40 to

50 90 parts by weight of a finely divided white coating pigment and from 10 to 60 parts by weight, solids basis, of polyvinyl acetate resin, substantially drying the coating, dampening the paper to impart thereto a moisture content of 7%-12%, supercalendering the coated paper, printing the paper on the coated surface, and applying a flexible, non-blocking film of wax over both surfaces of the paper, the amount of applied wax being sufficient, in conjunction with said coating, to enable a strong bond to be produced

55 between the exposed waxed areas of the paper with heat-sealing, whereby, when such heat-sealing takes place at a temperature high enough to melt said wax and soften the polyvinyl acetate resin, said coating and said wax will interact to produce a bond which will resist delamination at temperatures as low as 10° F.

6. The process of claim 5 wherein the wax is selected from the group consisting of paraffin wax, microcrystalline wax, and combinations thereof, and contains up to 15% by weight of polyethylene.

7. The process of claim 5 wherein the amount of pigment is from 75 to 87 parts, the amount of polyvinyl acetate is from 13 to 25 parts by weight, solids basis, and the viscosity of the adhesive composition is 250-1500 centipoises.

8. A coated heat-sealable wrapper for use in wrapping

frozen foodstuffs, comprising a sheet of paper having on an entire surface thereof a pigmented coating consisting essentially of a mixture of from 40 to 90 parts by weight of a finely divided coating pigment and from 10 to 60 parts, on a dry weight basis, of polyvinyl acetate resin, the amount of said coating being from 0.5 to 6 pounds per ream 3,000 sq. ft. of the paper, and having a flexible, non-blocking film of wax covering the entire coated surface of said sheet, the amount of wax being sufficient to interact with the polyvinyl acetate resin under heat-sealing to form a strong bond resisting delamination at temperatures as low as about 10° F.

9. A heat-sealable wrapper as described in claim 8, the wax in said film on the coated sheet being selected from the group consisting of paraffin wax, microcrystalline wax, and combinations thereof, and containing up to 40% by weight of polyethylene. 15

10. A coated, heat-sealable wrapper for use in wrapping frozen foodstuffs comprising a sheet of paper having a coating over one entire surface, said coating consisting essentially of a mixture of from 75 to 87 parts of white coating pigment and from 13 to 25 parts by weight, solids basis, of polyvinyl acetate resin, the amount of said coating being from 0.5 to 6 pounds per ream 3,000 sq. ft. of the paper, at least the coated surface of the paper being 20 covered by a flexible film of wax selected from the group consisting of paraffin wax, microcrystalline wax, and combinations thereof, and containing up to 15% by weight of polyethylene, said wrapper being characterized by forming, upon heat-sealing, a bond resisting delamination at 25 temperatures as low as 10° F. 30

11. A heat-sealable wrapper of claim 10, wherein the amount of wax is from about 8 to 25 pounds per ream of the paper.

5 12. A heat-sealable wrapper of claim 10, wherein the basis weight of the paper is from 20 to 35 pounds per ream, the amount of said coating is from 1.5 to 3 pounds per ream, the film of wax consists of 50-80% paraffin wax, 15-45% microcrystalline wax and 5-15% polyethylene, the percentages being expressed by weight, and 10 the amount of wax is from about 10 to 15 pounds per ream.

#### References Cited in the file of this patent

#### UNITED STATES PATENTS

|           |             |               |
|-----------|-------------|---------------|
| 2,306,046 | Duggan      | Dec. 22, 1942 |
| 2,394,254 | Noble       | Feb. 5, 1946  |
| 2,402,605 | Cowen       | June 25, 1946 |
| 2,406,990 | Borden      | Sept. 3, 1946 |
| 2,424,386 | Czeczwitzka | July 22, 1947 |
| 2,520,900 | Frost       | Sept. 5, 1950 |
| 2,529,060 | Trillich    | Nov. 7, 1950  |
| 2,609,317 | Vogt        | Sept. 2, 1952 |
| 2,656,286 | Fisher      | Oct. 23, 1953 |
| 2,720,467 | Franké      | Oct. 11, 1955 |
| 2,720,496 | Bushnell    | Oct. 11, 1955 |
| 2,733,225 | Smith       | Jan. 31, 1956 |
| 2,791,570 | Backlund    | May 7, 1957   |
| 2,803,612 | Moyer       | Aug. 20, 1957 |
| 2,808,382 | Jahoitis    | Oct. 1, 1957  |